

1

3,178,368  
**PROCESS FOR BASIC SULFURIZED METAL PHENATES**

Walter W. Hanneman, El Cerrito, Calif., assignor to California Research Corporation, San Francisco, Calif., a corporation of Delaware  
 No Drawing. Filed May 15, 1962, Ser. No. 194,996  
 5 Claims. (Cl. 252—33.4)

This invention pertains to a new process whereby highly basic sulfurized metal phenates are prepared. In particular, this process pertains to the manufacture of overbased sulfurized alkaline earth metal alkyl phenates.

Basic sulfurized alkaline earth metal alkyl phenates are used as compounding agents in lubricating oils to neutralize harmful acids, to inhibit corrosion, piston ring sticking and gum formation in internal combustion engines resulting from oxidation of the lubricating oil and oxidation polymerization of the engine fuel residues.

For many years, metal salts of phenolic materials have been used as additives for mineral lubricating oil compositions used in the lubrication of internal combustion engines. In combination with numerous other additives, the metal phenates improve the detergency characteristics of the lubricating oil, reduce engine wear, minimize the formation of harmful deposits on engine parts, and improve the resistance of the oil to oxidation.

Numerous attempts have been made to prepare oil-soluble sulfurized alkaline earth metal alkyl phenates which have the detergent characteristics of the metal phenates, and, in addition thereto, the property of neutralizing larger amounts of acidic bodies than possible with the presently available "normal" or "basic" sulfurized alkaline earth metal phenates. By the particular process described herein, it is possible to prepare overbased sulfurized alkaline earth metal alkyl phenates which can neutralize large amounts of acidity than possible with phenates available heretofore.

By the use of the term herein, "normal sulfurized alkaline earth metal phenates" refer to the metal phenates wherein the mole ratio of metal to the phenol nucleus is about 1:2, such as



wherein R represents the alkyl substituent radicals on the benzene ring, and M is an alkaline earth metal. The sulfur (—S—) is attached to both of the benzene rings.

The term "basic carbonated sulfurized alkaline earth metal phenates" refers to sulfurized alkaline earth metal phenates having base ratios in excess of 1.2; that is, the percent of the total alkaline earth metal to the metal of the normal phenate is greater than 20% in excess of the metal of the normal sulfurized alkaline earth metal phenates. A metal phenate having a base ratio of "1" is a neutral (a normal) phenate.

It is a particular advantage of this invention, that by the process described, "basic" carbonated sulfurized alkaline earth metal phenates having metal contents greater than 20% in excess of the metal present in the corresponding sulfurized normal alkaline earth metal phenates can be prepared. In particular, the base ratios of the resulting basic phenates have values from 1.2 to 4.5 or higher.

The overbased carbonated sulfurized alkaline earth metal phenates described herein are particularly useful when incorporated in lubricating oil compositions for diesel engines.

It is a primary object of this invention to set forth a new method of preparing highly overbased carbonated sulfurized alkaline earth metal phenates.

2

In accordance with this invention, it has been discovered that oil-soluble overbased carbonated sulfurized alkaline earth metal phenates can be prepared by the reaction of alkyl phenols with alkaline earth metal oxides or hydroxides, followed by carbonation with  $\text{CO}_2$  in the presence of glycol, sulfonates, and a high molecular weight alcohol. It is essential to the process described herein that the reaction mixture contains (1) a sulfonate, (2) ethylene glycol, and (3) a high molecular weight alcohol. Furthermore, for the satisfactory use as a lubricating oil additive of the final overbased sulfurized alkaline earth metal phenates, it is essential that the final basic phenate-oil blend contain the sulfonate, and it is desirable that the final oil blend contains a portion of the high molecular weight alcohol.

Briefly, the process of this invention comprises blending, then heating with agitation, a mixture of an alkyl phenol, a sulfonate, a high molecular weight alcohol, lubricating oil, and sulfur. Hydrated lime (or  $\text{CaO}$ ) is then added to this blend. The mixture is then heated, and ethylene glycol is added. Water of reaction is removed; the mixture is cooled, and carbon dioxide is added. Uncombined  $\text{CO}_2$  is removed, and the reaction vessel is heated to remove ethylene glycol, water, and high molecular weight alcohol.

Alkyl phenols which are used herein in the reaction mixture are represented by the formula:



wherein A is an "essentially hydrocarbon" aromatic radical, preferably a benzene radical, R is a straight-chain or branched-chain, saturated or unsaturated essentially hydrocarbon radical having from 4 to 30 carbon atoms and  $a$  is a number having a value from 1 to 2. The total number of carbon atoms for R has a minimum value of 8. Thus, when  $a$  is 1, the minimum number of carbon atoms in R is 8.

Examples of suitable hydrocarbonaceous radicals include alkyl radicals, such as butyl, hexyl, octyl, decyl, dodecyl, hexadecyl, eicosyl, tricosyl radicals; radicals derived from petroleum hydrocarbons, such as white oil, wax, olefin polymers (e.g., polypropylene and polybutylene), etc.

The basic sulfonates used herein contain from 0% to 300% of metal in excess of the metal of normal sulfonates, that is, essentially neutral, metal sulfonates. The basic sulfonates used herein are derived from neutral sulfonates represented by the formula:



wherein R is a high molecular weight straight-chained or branched-chain saturated or unsaturated essentially hydrocarbonaceous radical having a molecular weight of about 150 to about 800; A is an aromatic radical, such as benzene, naphthalene, anthracene, etc.;  $a$  is a number having the value of 1 to 4; and M is an alkaline earth metal.

As the metal, the term "alkaline earth metals," includes preferably calcium, barium, and strontium; calcium is particularly preferred.

Examples of suitable hydrocarbonaceous radicals are the following: dodecane, hexadecane, eicosane, triacontane radicals; radicals derived from petroleum hydrocarbons such as white oil, wax, olefin polymers (e.g., polypropylene and polybutylene, etc.). The sulfonic acids used in preparing the basic sulfonates of this invention also include the oil-soluble sulfonic acids obtained from petroleum, such as the "mahogany" acids, and the synthetic sulfonic acids prepared by various methods of synthesis (e.g., sulfonic acids prepared by reacting a chlorinated white oil with benzene, using hydrofluoric acid as

the catalyst, then treating the resulting white oil alkylated benzene with chlorosulfonic acid or fuming sulfuric acid to form a white oil benzene sulfonic acid).

The metal sulfonates are exemplified as follows: calcium white oil benzene sulfonate, barium white oil benzene sulfonate, calcium dipolypropylene benzene sulfonate, barium dipolypropylene benzene sulfonate, calcium mahogany petroleum sulfonate, barium mahogany petroleum sulfonate, calcium triacontyl benzene sulfonate, barium triacontyl benzene, etc.

The high molecular weight alcohol, which is used in amounts no more than 75% by weight of the alkyl phenol charged, preferably 10% to 50%, are those monohydric alcohols containing from 8 to 18 carbon atoms. These alcohols are exemplified as follows: octyl alcohol, decyl alcohol, dodecyl alcohol, tridecyl alcohol, tetradecyl alcohol, cetyl alcohol, etc.

In the process described herein, a lubricating oil may be used as a reaction medium. Thus, by such use of a lubricating oil, oil concentrates of the desired highly basic carbonated sulfurized metal phenates can be obtained. Such lubricating oils include a wide variety of lubricating oils, such as naphthenic base, paraffin base and mixed base lubricating oils, other hydrocarbon lubricants, e.g., lubricating oils derived from coal products and the synthetic oils, e.g., alkylene polymers (such as polymers of propylene, butylene, etc., and the mixtures thereof); alkylene oxide type polymers, e.g., alkylene oxide polymers prepared by polymerizing the alkylene oxides, e.g., propylene oxide, etc., in the presence of water or alcohols (e.g., ethyl alcohol); carboxylic acid esters, for example, those which are prepared by esterifying such carboxylic acids as adipic acid, azelaic acid, subaric acid, sebacic acid, alkenyl succinic acid, fumaric acid, maleic acid, etc. with alcohols such as butyl alcohol, hexyl alcohol, 2-ethylhexyl alcohol, and pentaerythritol; alkyl benzenes, polyphenyls; polymers of silicon; etc.

The several components which are used in this process are used in certain proportions with respect to each other. For each molal quantity of alkyl phenol, it is desirable to use from 0.01 mole to 1 mole of sulfonate, preferably 0.01 mole to 0.05 mole, and from 0.1 mole to 1.5 mole of high molecular weight alcohol, preferably tridecyl alcohol.

The amount of elemental sulfur present in the reaction mixture is such that the mol ratio of sulfur to alkaline earth metal of the basic substance is from 0.25 to 4.0. It is preferred that the mol ratio is in the range of 0.5 to 1.5.

The amount of alkaline earth metal oxide or hydroxide which is used is that amount which will be sufficient to give a base ratio of 1.2 to 4.5, preferably 1.5 to 3.5. The amount of alkaline earth metal oxides or hydroxide used in the reaction depends on the amount of metal desired in the product in excess of that of the normal phenate. Normally, in the preparation of basic carbonated sulfurized phenates a slight excess (e.g., 5 mole percent excess) of calcium oxide or hydroxide is used in the reaction mixture over that desired in the final basic phenate product.

The carbon dioxide used is from 300 mole percent to 10 mole percent, preferably 150 mole percent to 10 mole percent of the alkyl phenol charged.

In the process of this invention, it is preferred to use ethylene glycol. The amount of glycol used will depend upon the amount of calcium oxide or hydroxide used.

A sufficient amount of glycol is employed to bring the reactants into efficient contact for substantial reaction in a reasonably short time; that is, the amount of glycol used is sufficient to dissolve a portion of each of the reactants and to cause substantial contact between said reactants. For this purpose it is beneficial to use certain ratios by weight of the alkaline earth metal oxide or hydroxide to glycol. The alkaline earth metal-glycol mole ratio may vary from 2 to 1 to about 0.25 to 1.0; preferably from 1 to 1 to about 0.5 to 1.

According to the process described herein, there is first formed a blend consisting of an alkyl phenol, a sulfonate, a high molecular weight alcohol, and an oil of lubricating viscosity. This mixture is then heated with agitation to temperatures from 150° F. to 190° F., followed by the addition of the sulfur and calcium hydroxide (or oxide). This blend is then heated to temperatures in the range of 250° F. to 300° F., and that temperature is maintained while ethylene glycol is slowly added. The water of reaction liberated after the addition of the glycol is then removed by heating to temperatures of about 340° F. The reaction mixture is cooled slightly, followed by carbonation by means of carbon dioxide at temperatures from 250° F. to 350° F. Any uncombined CO<sub>2</sub> is then removed. The reaction blend is then heated for 2 to 10 hours at temperatures ranging from 300° F. to 390° F., during which heating the absolute pressure is reduced to 40-50 mm. Hg to remove glycol. In certain instances, some of the high molecular weight alcohols may be removed along with the ethylene glycol. However, whether or not any or all of the high molecular weight alcohol is removed, the resulting lubricating oil composition is highly effective for its intended purpose. When the particularly preferred high molecular weight alcohol is used, that is, tridecyl alcohol, it is beneficial that at least 50%, by weight, remain in the lubricating oil composition. However, with this preferred alcohol, the final lubricating oil composition may contain from 30% to 50%, by weight, of the original charge of the tridecyl alcohol. Thus, the high molecular weight alcohol may be removed in its entirety or amounts up to 100% of the initial charge may remain in the final composition.

The examples hereinbelow illustrate the process of this invention.

#### EXAMPLE I

##### *Preparation of basic sulfurized carbonated calcium alkyl phenate*

A mixture of 4,170 pounds of an alkyl phenol having a hydroxyl number of 184 wherein the alkyl radical was derived from a polypropylene having an average of 12 carbon atoms, 508 gallons of a California refined base oil having viscosities of 130 SSU at 100° F., 436 pounds of a basic calcium sulfonate containing 40% calcium in excess of that amount for a neutral sulfonate (i.e., the base ratio was 1.4:1), and 1294 pounds of tridecyl alcohol was heated to 180° F. with agitation. Sulfur, 854 pounds, was charged to the vessel with the temperature maintained at 180-190° F. Hydrated lime, 1974 pounds, was added to the blend. The temperature of the reaction mixture was increased to 260° F. Unheated ethylene glycol, 134 gallons, was added slowly to the reaction mixture, which was kept at a temperature of 260-270° F. for the glycol addition. The reaction mixture was then heated to 340° F. to remove water.

With rapid agitation of the reaction mixture 574 pounds of CO<sub>2</sub> was added at a rate of 100 pounds per hour at an initial temperature of 330° F. Uncombined CO<sub>2</sub> was removed. The mixture was heated to 390° F. at an absolute pressure of approximately 40 mm. Hg to remove, by distillation, water, ethylene glycol, and tridecyl alcohol. The remaining lubricating oil blend contained 9.72%, by weight, calcium.

As noted hereinabove, it is desirable that the final lubricating oil composition have a high basicity. In the process described, it is desirable that the initial amount of alkyl phenol be from 20% to 45%, by weight, based on the final composition, preferably from 25% to 35%, by weight. The lubricating oil reaction medium is used in amounts from 15% to 50%, by weight, based on the finished composition, preferably from 20% to 30%, by weight.

The metal sulfonate used in the example hereinabove was a concentrate consisting of 46.4% by weight of a mineral lubricating oil and 53.6% by weight of a calcium

petroleum sulfonate wherein the petroleum radical was derived from a mineral oil having a viscosity of 500 SSU at 100° F. The calcium content of the oil concentrate was 11.4% by weight, and the base ratio was 1.4.

I claim:

1. A process of preparing sulfurized basic alkaline earth metal carbonated alkyl phenate comprising forming a blend comprising a petroleum lubricating oil, an alkyl phenol wherein said alkyl radical has from 4 to 30 carbon atoms and the total number of carbon atoms in the alkyl groups is at least 8, an alkaline earth metal alkyl aryl sulfonate in an amount of from 0.01 to 1 mol per mol of said alkyl phenol and an aliphatic saturated monohydric alcohol having from 8 to 18 carbon atoms in an amount of from 10 to 75% by weight of said alkyl phenol, heating said blend to temperatures in the range of 150° F. to 190° F., adding thereto a basic substance selected from the group consisting of alkaline earth metal hydroxide and alkaline earth metal oxide in amount necessary to give a base ratio of from 1.2 to 4.5 for said basic alkaline earth metal carbonated alkyl phenate, and sulfur in an amount such that the mol ratio of sulfur to basic substance has a value from 0.25 to 4, heating said blend to temperatures in the range of 250° F. to 300° F., and at that temperature, adding unheated ethylene glycol thereto in amount such that the mole ratio of basic substance to ethylene glycol is from about 2:1 to about 0.25:1, removing the resulting water of reaction by heating to temperatures of about 340° F., while maintaining temperatures no lower than 250° F., adding carbon dioxide in amount of 10 mol percent to 300 mol percent of said alkyl phenol, maintaining the temperature of the reaction mixture at temperatures of 300° F. to 390° F. at reduced pressure to remove ethylene glycol.

2. A process of preparing a sulfurized basic alkaline earth metal carbonated alkyl phenate comprising forming a blend comprising a petroleum lubricating oil, an alkyl phenol wherein said alkyl radical is derived from a polypropylene having an average of 12 carbon atoms, an alkaline earth metal alkyl aryl sulfonate in an amount of from 0.01 to 1 mol per mol of said alkyl phenol, an aliphatic saturated monohydric alcohol having from 8 to 18 carbon atoms in amount of from 10% to 75% by weight of said alkyl phenol, heating with agitation to 180° F., while maintaining temperatures in the range of 180 to 190° F., adding thereto a basic substance selected from the group consisting of alkaline earth metal hydroxide and alkaline earth metal oxide in amount necessary to give a base ratio for the aforesaid carbonated alkyl phenate of from 1.2 to 4.5 and sulfur in an amount such that the mol ratio of sulfur to alkyl phenol has a value from 0.25 to 4, heating with agitation to 260° F., and while maintaining the reaction mixture at temperatures of 260-270° F., adding unheated ethylene glycol thereto in amount such that the mol ratio of basic substance to ethylene glycol is from 2:1 to about 0.25:1, heating to a temperature of about 340° F. to remove water of reaction, adding carbon dioxide in an amount of from 10 mol percent to 300 mol percent of said alkyl phenol, followed by heating to temperatures of 390° F. at reduced pressure to remove ethylene glycol and at least 50% of the original charge of said alcohol.

3. A process of preparing sulfurized basic alkaline earth metal carbonated alkyl phenate comprising forming a blend comprising from 20% to 30% by weight, based on the final composition, of a petroleum lubricating oil, from 20% to 45% by weight of an alkyl phenol wherein said alkyl radical has from 4 to 30 carbon atoms and the total number of carbon atoms in the alkyl groups is at least 8, an alkaline earth metal alkyl aryl sulfonate in an amount of from 0.01 to 1 mol per mol of said alkyl phenol and an aliphatic saturated monohydric alcohol having from 8 to 18 carbon atoms in an amount of from 10% to 75% by weight of said alkyl phenol,

heating said blend to temperatures in the range of 150° F. to 190° F., adding thereto a basic substance selected from the group consisting of alkaline earth metal hydroxide and alkaline earth metal oxide in amount necessary to give a base ratio of from 1.2 to 4.5 for said basic alkaline earth metal carbonated alkyl phenate, and sulfur in an amount such that the mol ratio of sulfur to basic substance has a value from 0.25 to 4, heating said blend to temperatures in the range of 250° F. to 300° F., and at that temperature, adding unheated ethylene glycol thereto in amount such that the mole ratio of basic substance to ethylene glycol is from about 2:1 to about 0.25:1, removing the resulting water of reaction by heating to temperatures of about 340° F., while maintaining temperatures no lower than 250° F., adding carbon dioxide in amount of 10 mol percent to 300 mol percent of said alkyl phenol, maintaining the temperature of the reaction mixture at temperatures of 300° F. to 390° F. at reduced pressure to remove ethylene glycol.

4. A process of preparing a sulfurized basic alkaline earth metal carbonated alkyl phenate comprising forming a blend comprising from 15% to 50% by weight, based on the final composition, of a lubricating oil, from 20% to 45% by weight of an alkyl phenol wherein said alkyl radical is derived from a polypropylene having an average of 12 carbon atoms, an alkaline earth metal alkyl aryl sulfonate in an amount of from 0.01 to 1 mol per mol of said alkyl phenol, an aliphatic saturated monohydric alcohol having from 8 to 18 carbon atoms in an amount of from 10% to 75% by weight of said alkyl phenol, heating with agitation to 180° F., and while maintaining the temperatures in the range of 180 to 190° F., adding thereto a basic substance selected from the group consisting of alkaline earth metal hydroxide and alkaline earth metal oxide in amount necessary to give a base ratio for the aforesaid carbonated alkyl phenate of from 1.2 to 4.5, and a sulfur in an amount such that the mol ratio of sulfur to alkyl phenol has a value from 0.25 to 4, heating said mixture with agitation to 260° F., and, while maintaining the reaction mixture at temperatures of 260-270° F., adding ethylene glycol thereto in amount such that the mol ratio of basic substance to ethylene glycol is from 2:1 to 0.25:1, heating said reaction mixture to a temperature of 340° F. to remove water of reaction, adding carbon dioxide at temperatures of from about 250° F. to about 300° F. in an amount of from 10 mol percent to 300 mol percent of said alkyl phenol, followed by heating to temperatures of 390° F. at reduced pressure to remove ethylene glycol and at least 50% by weight of the original charge of said monohydric alcohol.

5. A process of preparing a sulfurized basic calcium carbonated alkyl phenate comprising forming a blend comprising from 20% to 30% by weight, based on the final composition, of a petroleum lubricating oil, from 25% to 35% by weight of an alkyl phenol wherein said alkyl radical is derived from a polypropylene having an average of 12 carbon atoms, a calcium alkyl aryl sulfonate in an amount of from 0.01 to 0.05 mol per mol of said alkyl phenol, an aliphatic saturated monohydric alcohol having from 8 to 18 carbon atoms in an amount of from 10% to 50% by weight of said alkyl phenol, heating with agitation to 180° F., and while maintaining temperatures of 180 to 190° F., adding thereto a basic substance selected from the group consisting of calcium hydroxide and calcium oxide in amount necessary to give a base ratio for the aforesaid carbonated alkyl phenate of from 1.2 to 4.5, and sulfur in an amount such that the mol ratio of sulfur to alkyl phenol has a value from 0.5 to 1.5; heating the reaction mixture with agitation to 260° F., and while maintaining the reaction mixture at a temperature in the range of 260 to 270° F., adding ethylene glycol thereto in amount such that the mol ratio of basic substance to ethylene glycol is from 2:1 to about 0.25:1, heating to a temperature of about

340° F., to remove water of reaction, adding carbon dioxide at temperatures of from about 250° F. to about 300° F. in an amount of from 10 mol percent to 150 mol percent of said alkyl phenol, followed by heating to temperatures of 390° F. at reduced pressure to remove ethylene glycol and at least 50% by weight of the original charge of said alcohol. 5

## References Cited by the Examiner

## UNITED STATES PATENTS

|           |       |                         |          |
|-----------|-------|-------------------------|----------|
| 2,119,114 | 5/38  | Richardson et al. ----- | 252—52   |
| 2,409,687 | 10/46 | Rogers et al. -----     | 252—42.7 |
| 2,409,726 | 10/46 | Winning et al. -----    | 252—52   |

10

|           |       |                        |            |
|-----------|-------|------------------------|------------|
| 2,483,505 | 10/49 | Rogers et al. -----    | 252—42.7   |
| 2,680,096 | 1/54  | Walker et al. -----    | 252—42.7   |
| 2,766,291 | 10/56 | Weissberg et al. ----- | 252—42.7 X |
| 3,036,971 | 5/62  | Otto -----             | 252—42.7   |

## FOREIGN PATENTS

|         |       |                |
|---------|-------|----------------|
| 727,655 | 4/55  | Great Britain. |
| 776,455 | 6/57  | Great Britain. |
| 821,397 | 10/59 | Great Britain. |

DANIEL E. WYMAN, Primary Examiner.

JULIUS GREENWALD, Examiner.